



US005703431A

**United States Patent** [19]

Itou et al.

[11] Patent Number: **5,703,431**[45] Date of Patent: **Dec. 30, 1997**[54] **DISPLAY SCREEN AND METHOD OF MANUFACTURING THE SAME**[75] Inventors: **Takeo Itou, Kumagaya; Hidemi Matsuda, Fukaya, both of Japan**[73] Assignee: **Kabushiki Kaisha Toshiba, Kawasaki, Japan**[21] Appl. No.: **579,609**[22] Filed: **Dec. 26, 1995**[30] **Foreign Application Priority Data**

Dec. 26, 1994 [JP] Japan ..... 6-322059

[51] Int. Cl.<sup>6</sup> ..... **H01J 29/10**[52] U.S. Cl. ..... **313/461; 313/463; 313/466; 313/473**[58] Field of Search ..... **313/461, 463, 313/466, 473**[56] **References Cited**

## U.S. PATENT DOCUMENTS

2,959,483 11/1960 Kaplan .  
 3,114,065 12/1963 Kaplan .  
 4,021,588 5/1977 Royce et al. ..... 313/466

|           |         |                      |         |
|-----------|---------|----------------------|---------|
| 4,251,610 | 2/1981  | Haven et al. ....    | 430/25  |
| 4,392,077 | 7/1983  | Libman ....          | 313/474 |
| 4,551,652 | 11/1985 | Compen et al. ....   | 313/466 |
| 5,045,750 | 9/1991  | Itou et al. ....     | 313/461 |
| 5,199,984 | 4/1993  | Jeong ....           | 313/466 |
| 5,340,673 | 8/1994  | Tateyama et al. .... | 430/23  |

**FOREIGN PATENT DOCUMENTS**

|           |         |                      |
|-----------|---------|----------------------|
| 0 322 200 | 6/1989  | European Pat. Off. . |
| 0 613 167 | 8/1994  | European Pat. Off. . |
| 54-000563 | 1/1979  | Japan .              |
| 5-266795  | 10/1993 | Japan .              |
| 5-275006  | 10/1993 | Japan .              |
| 2 240 213 | 7/1991  | United Kingdom .     |

*Primary Examiner*—Sandra L. O’Shea*Assistant Examiner*—Vip Patel*Attorney, Agent, or Firm*—Cushman Darby & Cushman IP Group of Pillsbury Madison & Sutro LLP[57] **ABSTRACT**

There is disclosed a display screen including a transparent substrate, color optical filters formed on the substrate, and a black matrix layer formed on the filters and consisting of black pigment particles. Phosphor layers are formed on the color optical filters on which the black matrix layer is formed.

**8 Claims, 4 Drawing Sheets**



FIG. 1

(PRIOR ART)



FIG. 2A



FIG. 2B



FIG. 2C



F I G. 4A



F I G. 4B



F I G. 4C



F I G. 4D



F I G. 4E



F I G. 4F





FIG. 5A



FIG. 5B



FIG. 6



FIG. 7

## DISPLAY SCREEN AND METHOD OF MANUFACTURING THE SAME

### BACKGROUND OF THE INVENTION

#### 1. Field of the Invention

The present invention relates to a display screen used in a color cathode ray tube.

The present invention particularly relates to a display screen having an optical color filter layer formed between a phosphor layer and a substrate, and a method of manufacturing the display screen.

#### 2. Description of the Related Art

A conventional color television tube used in practice includes an envelope. The envelope includes a panel having a phosphor screen formed on its inner surface and a funnel continuous with this panel. An electron gun unit assembly is arranged in the neck portion of the funnel. Electron beams emitted from the electron gun are deflected and scanned by a magnetic field generated by a deflection yoke mounted on the outer surface of the envelope, thereby forming an image.

This phosphor screen has a black matrix formed on the inner surface of a faceplate, consisting of black pigment particles, and having circular, rectangular, or stripe-shaped holes at predetermined positions. The phosphor screen also has circular, rectangular, or stripe-shaped phosphor layers which fill the holes.

A so-called tint panel or dark tint panel is generally used as a low-transmittance faceplate to attenuate external light reflection components and increase the contrast ratio in a color television tube. When this faceplate is used, emission from the phosphors is attenuated in addition to the attenuation of the external light reflection components, resulting in inconvenience.

A technique shown in Jpn. Pat. Appln. KOKAI Publication No. 5-275006, or the like, has recently received a great deal of attention. In this technique, filter patterns constituted by phosphor layers, and pigment layers corresponding to the emission colors of the respective phosphors of the phosphor layers are formed between the phosphor layers and the faceplate to suppress the reflection at the face of the phosphor layers. Thus, the contrast is increased.

FIG. 1 is a schematic sectional view for explaining a conventional display screen. As shown in FIG. 1, to manufacture a phosphor screen with filters in which red, green, and blue filters RF, GF, BF, and red, green, and blue emission phosphor layers RP, GP, and BP are formed in the holes of a black matrix BM. The step of forming the filters RF, GF, and BF on the front surfaces of the phosphor layers RP, GP, and BP, i.e., on the faceplate 10 side, is required in addition to the conventional manufacturing process of the phosphor screen. Most of the methods recently proposed for this purpose form a filter pattern prior to formation of the phosphor layers, but after the black matrix BM is formed on the inner surface of the faceplate.

As another method of suppressing the reflection described above, an optical interference film corresponding to emission of phosphors is formed between phosphor layers and a faceplate, as shown in Jpn. Pat. Appln. KOKAI Publication No. 54-563. In view of the number of manufacturing steps and cost, however, a method of forming pigment particle layers in correspondence with the respective phosphors is superior to the above method.

According to the method of forming a filter pattern consisting of pigment particle layers between phosphor layers and a faceplate, even if a high-transmittance faceplate

is used, the contrast and emission brightness can be theoretically increased. An irregular reflection component of black pigment particles can not be suppressed. However an expected effect of suppressing external light reflection cannot be obtained if the optical filter pattern is simply formed between the phosphor layers and the faceplate in the holes. For this reason, sufficiently high brightness and contrast levels cannot be desirably obtained.

In the conventional method of manufacturing the phosphor screen with filters, the black matrix under the pigment layers peels off the substrate during the manufacture, and more specifically, at the stage in which filter layers are formed on the substrate having the black matrix and patterned.

### SUMMARY OF THE INVENTION

The present invention has been made in consideration of the conventional problems described above, and has as its object an efficient suppression of external light reflection on a filter substrate with a black matrix and a color television tube.

It is another object of the present invention to provide a method of manufacturing a filter substrate and a color television tube free from the peeling of a black matrix during the manufacture.

According to the first aspect of the present invention, there is provided a display screen comprising:

a transparent substrate;

30 optical filter layers containing color pigment particles having an average particle size of 0.2  $\mu\text{m}$  or less and formed on the transparent substrate as rectangular or circular dots or stripes;

35 a black matrix layer containing black pigment particles having an average particle size of 0.2 to 5  $\mu\text{m}$  and formed to cover peripheral regions of the filter layers except for central portions thereof; and

40 phosphor layers formed on the optical filter layers and having an emission color corresponding to a color of a pigment contained in the optical filter layers.

According to the second aspect of the present invention, there is provided a method of manufacturing a display screen, comprising the step of:

45 coating and drying a color pigment dispersion containing color pigment particles having an average particle size of 0.2  $\mu\text{m}$  or less on a transparent substrate to form a color pigment layer, and patterning the color pigment layer to form optical pigment layers as rectangular or circular dots or stripes;

50 coating and drying a black pigment dispersion containing black pigment particles having an average particle size of 0.2 to 5  $\mu\text{m}$  on the color pigment layers to form a black pigment layer, and patterning the black pigment layer to partially remove the black pigment layer except for peripheral regions of the pigment layers so as to expose at least central portions of the optical filter layers, thereby obtaining a black matrix layer covering the peripheral regions of the color optical filter layers; and

55 coating a slurry containing a phosphor on the color pigment layers to form a phosphor slurry layer, and patterning the phosphor slurry layer to optionally form phosphor layers having an emission color corresponding to a color of a pigment containing the optical filter layers on the optical filter layers.

60 According to the present invention, since the filter layers consisting of fine particle pigments are formed between the substrate and the black matrix consisting of black pigment

particles, components irregularly reflected by the black pigment particles can be suppressed to improve the contrast characteristics of the display screen with respect to external light. Therefore, when the display screen of the present invention is used, a color cathode ray tube which is excellent in brightness and contrast can be obtained.

According to the manufacturing method of the present invention, materials are patterned from the one having a smaller particle size. The lower pattern already formed in the manufacturing process will not peel off in patterning an upper layer, thereby providing an excellent display screen and an excellent color cathode ray tube.

Additional objects and advantages of the invention will be set forth in the description which follows, and in part will be obvious from the description, or may be learned by practice of the invention. The objects and advantages of the invention may be realized and obtained by means of the instrumentalities and combinations particularly pointed out in the appended claims.

#### BRIEF DESCRIPTION OF THE DRAWINGS

The accompanying drawings, which are incorporated in and constitute a part of the specification, illustrate presently preferred embodiments of the invention and, together with the general description given above and the detailed description of the preferred embodiments given below, serve to explain the principles of the invention.

FIG. 1 is a schematic sectional view for explaining a conventional display screen;

FIG. 2A is a schematic plan view showing a display screen according to the present invention;

FIG. 2B is a sectional view of the display screen along the line X—X in FIG. 2A;

FIG. 2C is a sectional view of the display screen along the line Y—Y in FIG. 2A;

FIGS. 3A to 3G are sectional views for explaining a method of manufacturing the display screen according to the present invention;

FIGS. 4A to 4F are sectional views for explaining another method of manufacturing the display screen according to the present invention;

FIG. 5A is a schematic plan view for explaining another display screen according to the present invention;

FIG. 5B is a sectional view of the display screen along the line C—C in FIG. 5A;

FIG. 6 is a schematic view showing a color cathode ray tube to which the display screen according to the present invention can be coated; and

FIG. 7 is a schematic sectional view for explaining a phosphor screen in FIG. 6.

#### DETAILED DESCRIPTION OF THE PREFERRED EMBODIMENTS

The present inventors examined the causes for the problems of a conventional display screen with filters, i.e., i) the failure of providing an expected effect of preventing external light reflection, and ii) easy peeling of a black matrix layer during the manufacture.

As for problem i), irregular reflection caused by pigment particles which form a black matrix was found to be noticeable with an increase in transmittance of a faceplate. High brightness and contrast levels which could be expected upon employment of filters could not be obtained due to this irregular reflection.

More specifically, since the pigment particles contained in the optical filter layers formed between the faceplate and the phosphor layers have an average particle size of about 0.2  $\mu\text{m}$ , or less irregular reflection caused by the particles does not occur. However, since the black pigment particles contained in the black matrix layer have a relatively large particle size of 0.2 to 5  $\mu\text{m}$ , the external light is irregularly reflected by the black matrix layer. This irregular reflection does not pose a problem in a conventional faceplate because its transmittance is low. With an increase in transmittance of the faceplate, irregular reflection in the black matrix layer is not attenuated and becomes noticeable.

In a conventional color cathode ray tube having a filter substrate and phosphor layers with filters, no countermeasure is taken for the black matrix layer serving as a non-emission portion. That is, no counter measure is taken to prevent irregular reflection in the black matrix layer. This is the cause for the failure of providing the expected effect of preventing external light reflection.

As for problem ii), the filter layers and the black matrix layer are found to have different forces based on film shrinkage during film drying, thereby causing the peeling of the black matrix during the manufacturing process.

This will be described below in detail.

The force based on film shrinkage during the film drying is represented by equation I below:

$$P=2\gamma r \quad \text{equation I}$$

where P is the shrinkage force,  $\gamma$  is the surface tension, and r is the radius of the air gap.

As the particle size decreases, the radius r of the air gap decreases. For this reason, it is found from equation I that the shrinkage force P increases with a decrease in particle size.

Since the average particle size of the pigment particles used in the optical filter layers falls within the range of about 0.20  $\mu\text{m}$  or less and the average particle size of the black pigment particles used in the black matrix layer falls within the range of 0.2 to 5  $\mu\text{m}$ , a large difference is present between the shrinkage forces of the black matrix layer and the optical filter layers. Therefore, the difference between the shrinkage forces of the black matrix layer and the optical filter layers is found to be the cause of peeling of the black matrix layer from the optical filter layers.

Judging from the above fact, the present inventors have confirmed that problems i) and ii) can be solved by implementing the arrangement so as to eliminate the influences of the shrinkage force of the optical filter layers and have reached the present invention.

According to the first aspect of the present invention, there is provided a display screen comprising:

a transparent substrate;  
optical filter layers containing color pigment particles having an average particle size of 0.2  $\mu\text{m}$  or less and formed on the transparent substrate as rectangular or circular dots or stripes;

a black matrix layer containing black pigment particles having an average particle size of 0.2 to 5  $\mu\text{m}$  and formed to cover peripheral regions of the filter layers except for central portions thereof; and

phosphor layers formed on the optical filter layers and having an emission color corresponding to a color of a pigment contained in the optical filter layers.

In a conventional display screen, a black matrix layer is directly formed on a faceplate, and no optical filter layers are present between the black matrix layer and the faceplate. In

the display screen according to the present invention, however, the optical filter layers are formed at least partially between the black matrix layer and the faceplate. These optical filter layers can suppress irregular reflection of external light on the black matrix layer. Therefore, a color cathode ray tube having this display screen can have higher contrast and brightness levels.

When the optical filter layers of the respective colors are formed as, e.g., circular dots, a gap is formed between the circles of the filter layers. The black matrix layer is directly formed on the substrate and no optical filter layer is present in this gap. Thus, the optical filter layer is formed partially between the black matrix layer and the faceplate. In contrast, when the optical filter layers of the respective colors are formed as, e.g., stripes so as to cover the entire surface of the substrate without any gap, the optical filters are interposed entirely between the black matrix layer and the substrate. Therefore, irregular reflection caused by the black pigment particles can be more effectively prevented on the entire surface of the substrate.

The second aspect of the present invention represents a method of manufacturing the display screen of the first aspect. There is provided a method of manufacturing a display screen, comprising the steps of:

coating and drying a color pigment dispersion containing color pigment particles having an average particle size of 0.2  $\mu\text{m}$  or less on a transparent substrate to form a color pigment layer, and patterning the color pigment layer to form color optical filter layers as rectangular or circular dots or stripes;

coating and drying a black pigment dispersion containing black pigment particles having an average particle size of 0.2 to 5  $\mu\text{m}$  on the color pigment layers to form a black pigment layer, and patterning the black pigment layer to partially remove the black pigment layer except for peripheral regions of the color optical filter layers so as to expose at least central portions of the optical filter layers, thereby obtaining a black matrix layer covering the peripheral regions of the color optical filter layers; and

coating a slurry containing a phosphor on the color optical filter layers to form a phosphor slurry layer, and patterning the phosphor slurry layer to optionally form phosphor layers having an emission color corresponding to a color of a pigment containing the optical filter layers on the optical filter layers.

The color optical filter layers are formed in units of colors by repeating the step of coating a dispersion including a color pigment and a resist to form a coating film, the step of exposing the coating film, and developing the exposed coating film. If the resultant color optical filter layers are formed as circular dots, they have gaps between themselves.

The color optical filter layers can also be formed by the following method. Assume that color optical filter layers of  $n$  colors are to be formed. Prior to coating of the first color pigment dispersion, a resist solution is coated on a substrate to form a resist film. The resist film is exposed and developed to form a resist film pattern in a region where the color optical filter layers of the second to  $n$ th colors are to be formed. The first pigment dispersion is coated and dried on the resist film pattern to form a coating film. A resist decomposition solution is coated on the first pigment dispersion coating film to remove the resist film pattern and the first color pigment dispersion coating film formed thereon in the region where the color optical filter layers of the second to  $n$ th colors are to be formed. Thus the substrate is exposed in this region.

The second pigment dispersion is coated on the exposed substrate to form a coating film. The coating film is exposed

and developed. The coating film is patterned into optical filter layers of the second color. Similarly, coating films up to the  $n$ th color are sequentially patterned until the color optical filter layers of the  $n$ th color are formed. In the resultant color optical filters, portions corresponding to the gaps between the color optical filter layers formed in the former method are buried with the first color optical filters. No gaps are formed in this latter method. If the optical filter layers are formed as circular dots, the display screen manufactured by the latter method can more effectively suppress irregular reflection caused by the black pigment particles than that manufactured by the former method.

The black matrix layer, for example, can be formed as follows.

15 A resist solution is coated to form a resist coating film. The resist coating film is exposed, developed, and patterned to form a resist layer pattern in a prospective phosphor layer formation region near the central portion of each color optical filter layer. A black pigment dispersion is coated on 20 the color optical filter layers, on which the resist layer pattern is formed, to form a black pigment layer. A resist decomposition agent is coated on the black pigment layer to remove the resist layer and the black pigment layer in the region where the phosphor layers are formed. As described 25 above, a portion near the central portion of each optical filter layer is exposed, and the black matrix layer can be formed to cover the peripheral portion of each color pigment layer.

In a conventional method, optical filter layers are formed on a black matrix layer. The black matrix layer formed under 30 the optical filter layers tend to peel off by the influence of a strong shrinkage force generated during coating and drying of the optical filter layers. According to the manufacturing method of the present invention, however, the pattern of the optical filter layers is formed prior to the formation of the black matrix layer. The black matrix layer is not adversely affected by the shrinkage force of the optical filter layers. A weak shrinkage force generated in coating and drying of the black matrix layer is not strong enough to cause peeling of the optical filter layers formed under the black matrix layer. 35 In other words, the film shrinkage force increases with a decrease in particle size. According to the manufacturing method of the present invention, a material having a larger film shrinkage force is formed first, thereby reducing the force that acts on the lower layer in patterning the upper 40 layer. As described above, according to the present invention, a display screen with filters can be obtained without the peeling of the black matrix film.

Color pigment particles used in the present invention have an average particle size of 0.005 to 0.2  $\mu\text{m}$  to obtain optical 45 filters capable of transmitting desired light and having sufficiently high transparency and good film formation properties. Scattering is decreased when the particle size of color pigment particles is 0.2, or less smaller particles among color pigment particles have the particle size of 0.005  $\mu\text{m}$ . Note that the desired particle size ranges within 0.01 to 0.15  $\mu\text{m}$ . Examples of the pigments are as follows.

Examples of the red pigment are: Sicotrans Red L-2817 (tradename), which has particle size of 0.01 to 0.02  $\mu\text{m}$  and is available from BASF, as a ferric oxide pigment, and 50 Chlomofartal Red A2B (tradename), which has a particle size of 0.01  $\mu\text{m}$  and is available from Ciba-Geigy) as an anthraquinone pigment. Examples of the blue pigment are: Cobalt Blue X (tradename), which has a particle size: 0.01 to 0.02  $\mu\text{m}$  and is available from Toyo Ganryo, as a cobalt 55 aluminate ( $\text{Al}_2\text{O}_3\text{—CoO}$ ) pigment; and Lionol Blue FG-7330 (tradename), which has a particle size of 0.01 and is available from Toyo Ink, as a phothalocyanine blue

5 pigment. Examples of the green pigment are Dyeroxide TM-Green #3320 (tradename), which has a particle size: 0.01 to 0.02  $\mu\text{m}$  and is available from DAINICHISEIKA COLOUR & CHEMICALS MFG. CO., LTD., as a  $\text{TiO}_2$ — $\text{NiO}$ — $\text{CoO}$ — $\text{ZnO}$  pigment, Dyeroxide TM-Green #3340 (tradename), which has a particle size of 0.01 to 0.02  $\mu\text{m}$  and is available from DAINICHISEIKA COLOUR & CHEMICALS MFG. CO., LTD., as a  $\text{CoO}$ — $\text{Al}_2\text{O}_3$ — $\text{Cr}_2\text{O}_3$ — $\text{TiO}_2$  pigment; Diperoxide TM-green #3420 (tradename), which has a particle size of 0.01 to 0.02  $\mu\text{m}$  and is available from DAINICHISEIKA COLOUR & CHEMICALS MFG. CO., LTD., as a  $\text{CoO}$ — $\text{Al}_2\text{O}_3$ — $\text{Cr}_2\text{O}_3$  pigment; Fastgen Green S (tradename), which has a particle size of 0.01  $\mu\text{m}$  and is available from DAINIPPON INK & CHEMICALS, INC., as a chlorinated phthalocyanine green pigment; and Fastgen Green 2YK (tradename), which has a particle size of 0.01  $\mu\text{m}$  and is available from DAINIPPON INK & CHEMICALS, INC., as a brominated phthalocyanine green pigment.

10 The second pigment particles as the black pigment particles preferably have an average particle size of 0.2 to 5  $\mu\text{m}$ , and can use graphite particles.

15 According to the method of the present invention, as described above, a fine particle pigment layer having a small particle size is formed in the manufacturing process of the phosphor screen. Even if the black pigment layer containing large particles is then formed and dried, and the resultant coating film is patterned, the underlying fine particle pigment layer pattern will not peel off. Thus, an excellent phosphor screen is obtained.

20 The present invention will be described in detail with reference to the accompanying drawings.

#### EXAMPLE 1

25 FIG. 2A is a schematic plan view showing a display screen in which optical filter layers as circular dots and a black matrix layer are formed on a substrate. FIGS. 2B and 2C are sectional views of the display screen along the lines X—X and Y—Y in FIG. 2A, respectively.

30 Referring to FIG. 2A, hatched lines represent a region where the black matrix layer is present, and portions surrounded by circles of dotted lines represent holes in which the black matrix layer is not present. Portions surrounded by circles of solid lines represent regions where optical filter layers as circular dots are formed. As shown in FIG. 2A, red, green, and blue filters RF, GF, and BF are formed adjacent to each other on a substrate 10. The red filter RF consists of a red pigment containing red iron oxide particles having an average particle size of 0.01  $\mu\text{m}$ . The green filter GF consists of a green pigment containing cobalt green particles having an average particle size of 0.01  $\mu\text{m}$ . The blue filter BF consists of a blue pigment containing cobalt blue particles having an average particle size of 0.01  $\mu\text{m}$ .

35 As shown in FIGS. 2B and 2C, a layer BM containing graphite particles is formed as a black matrix layer on the optical filter layers BF, GF, and RF consisting of such color pigment particles. The black matrix layer BM is not formed in the central portions of the dot-like pigment layers RF, GF, and BF, i.e., the circular regions indicated by the broken lines to define holes 20, as shown in FIG. 2B. The black matrix BM is formed to cover the peripheral portions of the color filters RF, GF, and BF and a portion between the color filters except for the holes 20.

40 As shown in FIG. 2C, the black matrix BM is formed on the substrate 10 in an inter-dot region which is not filled even if the pigment particle layers as circular dots are densely arranged adjacent to each other. In this case, as can be apparent from FIGS. 2A and 2C, at least the region between

45 the circle indicated by the solid line and the circle indicated by the broken line has a structure in which the corresponding optical filter layer is located between the black matrix layer BM and the substrate 10.

50 With this arrangement, the covering ratio of the fine particle pigment layers which cover the front surface, i.e., the substrate side of the black matrix is much higher in the display screen of the present invention than that of the conventional structure, 0%.

55 A method of manufacturing a display screen according to the present invention will be described below.

60 FIGS. 3A to 3G are sectional views for explaining a method of manufacturing the display screen according to the present invention.

65 As shown in FIG. 3A, red iron oxide particles are prepared as a red pigment, and an ammonium dichromate/poval photoresist is mixed therewith to prepare a red pigment dispersion. The resultant red pigment dispersion is coated on one surface of a clean transparent substrate 10 and dried. The red dot positions of the resultant coating film are exposed and developed to form red filters RF.

70 Cobalt blue is prepared as a blue pigment, and an ammonium dichromate/poval photoresist is mixed therewith to prepare a blue pigment dispersion. The resultant blue pigment dispersion is coated on the surface of the substrate and dried. The blue dot positions of the resultant coating film are exposed and developed to form blue filters BF, as shown in FIG. 3B. Following the same procedures as described above, cobalt green is used as a green pigment to form green filters GF, as shown in FIG. 3C.

75 As shown in FIG. 3D, a bisazido/polyvinyl pyrrolidone photoresist is coated on the color filters RF, GF, BR to form a resist layer 32. The green, blue, and red dot positions are exposed and developed by the conventional method to form resist patterns 34R, 34G, and 34B, as shown in FIG. 3E. As shown in FIG. 3F, a graphite suspension 40 is coated on the resultant structure to form a coating film. The resist patterns 34R, 34G, and 34B are decomposed in a treatment with a resist decomposition agent. The resist patterns 34R, 34G, and 34B and the graphite suspension coating film formed thereon are removed by development in which water is sprayed at high pressure of about 4 to 8 kg/cm<sup>2</sup>. As shown in FIG. 3G, a black matrix layer BM is formed except for the green, blue, and red dot positions, i.e., except for holes 20.

80 The red pigment dispersion, the blue pigment dispersion, and the green pigment dispersion can be obtained by the following composition.

#### Red pigment dispersion

|                                           |         |
|-------------------------------------------|---------|
| Sicotrans Red L-2817                      | 8 g     |
| POVAL EG-40                               | 0.9 g   |
| (available from NIHON GOSEI KAGAKU KOGYO) |         |
| Ammonium dichromate                       | 0.05 g  |
| (available from KANTO KAGAKU)             |         |
| Water                                     | 120 g   |
| dispersant                                | balance |

#### Blue pigment dispersion

|                                           |         |
|-------------------------------------------|---------|
| Cobalt Blue X                             | 8 g     |
| POVAL EG-40                               | 0.9 g   |
| (available from NIHON GOSEI KAGAKU KOGYO) |         |
| Ammonium dichromate                       | 0.05 g  |
| (available from KANTO KAGAKU)             |         |
| Water                                     | 50 g    |
| dispersant                                | balance |

## Green pigment dispersion

|                                           |         |
|-------------------------------------------|---------|
| Dyepynoxide TM-Green #3320                | 70 g    |
| POVAL EG-40                               | 0.9 g   |
| (available from NIHON GOSEI KAGAKU KOGYO) |         |
| Ammonium dichromate                       | 0.05 g  |
| (available from KANTO KAGAKU)             |         |
| Water                                     | 70 g    |
| dispersant                                | balance |

Any dispersant which can make pigment particles dispersed can be used in the pigment dispersion. An anionic type, nonionic type dispersant or a mixture thereof can be used as the dispersant.

Example of the anionic type dispersants are acrylic base, acryl-styrene type polymer, acryl copolymer, polycarbonates, condensates of naphthalene formalinsulfonate and polyoxyethylenealkylethersulfate. Example of the nonionic type dispersant are polyoxyethylenelaurylether, polyoxyethylene derivative, polyoxyalkylenealkylether, polyoxyethylenenonylphenylether polyoxyethylenesorbitanmonolaurylate.

When a filter substrate was actually formed by the method described above, no pattern peeling occurred during the formation process.

Since the fine particle pigment layers were formed between the black matrix layer and the substrate in the resultant display screen, irregular reflection caused by the black pigment particles was reduced, and the contrast characteristics of the filter substrate were improved.

Examples of a photoresist are chromates/POVAL type, diazonium salts/POVAL type, stilbazol type and chromates/casein type.

Examples of the resist decomposition agent used in the present invention are acids such as  $H_2SO_4$ , sulfamic acid, and peroxide such as  $H_2O_2$ ,  $MnKO_4$ ,  $KIO_4$ , and  $NaIO_4$ .

If required, coroidal silica and water glass can be applied to the color filter layers before BM is formed. Additionally, a silane coupling agent can be coated to improve adhesive force of BM particles.

## EXAMPLE 2

The black pigment layers are formed in the gaps between the pigment layer dots in Example 1. However, a substrate may be covered with fine particle pigment layers, and a black pigment layer may be formed thereon. FIGS. 4A to 4F are sectional views for explaining another method of manufacturing the display screen of the present invention.

An ammonium dichromate/poval photoresist is coated on one surface of a clean transparent substrate 10 to form a coating film. Resist patterns 50G and 50B shown in FIG. 4A are left at the positions where the blue and green dot positions are exposed and developed.

As shown in FIG. 4B, a red pigment fine particle dispersion using red iron oxide serving as a red pigment is coated and dried, and then the resist patterns 50G and 50B are removed using a decomposition agent. As shown in FIG. 4C, red filters RF are formed in regions except for the green and blue dot positions.

A blue pigment fine particle dispersion obtained by mixing an ammonium dichromate/poval photoresist in cobalt blue serving as a blue pigment is coated to expose and develop the blue dot positions, thereby forming blue filters BF shown in FIG. 4D. Following the same procedures as

described above, cobalt green is used to form green filters GF, as shown in FIG. 4E.

A bisazido/polyvinyl pyrrolidone photoresist is coated to form a resist layer. The green, blue, and red dot positions are exposed and developed by the conventional method to form resist patterns. A black matrix BM is formed at positions except for the green, blue, and red dot positions, i.e., except for holes 20, through coating of a graphite suspension, treatment with a decomposition agent, and development.

As shown in FIG. 4F, in the resultant filter substrate, the filters RF, GF, and BF consisting of fine particle pigments are formed on the substrate 10 side of the black matrix BM without forming gaps between the adjacent filters. Therefore, irregular reflection caused by the black pigment particles constituting the black matrix can be further reduced as compared with Example 1.

## EXAMPLE 3

Examples 1 and 2 have exemplified fine particle pigment layers as circular dots. Example 3 exemplifies fine particle pigment layers having another shape.

FIG. 5A is a schematic view of a display screen having stripe-shaped black matrices when viewed from the substrate side. Hatched lines represent regions in which the black matrices are present. FIG. 5B is a sectional view of the display screen along the line C—C in FIG. 5A. As shown in FIGS. 5A and 5B, stripe-shaped filter layers RF, GF, and BF are formed on a substrate 10 adjacent to each other without forming gaps between the adjacent filter layers in this display screen. Stripe-shaped black matrices are formed on the filter layers RF, GF, and BF so as to cover the peripheral regions of the filter layers except for their central portions.

A filter substrate of Example 3 can be manufactured following the same procedures as in Example 1 or 2, and is free from pattern peeling during the formation process.

The ratio of the fine particle pigment layers present between the black pigment particles and the substrate, i.e., the covering ratio, in Example 3 is higher than that in Example 1. An increase in contrast in Example 3 is larger than that in Example 1.

## EXAMPLE 4

Example 4 in which the present invention is coated on a color cathode ray tube will be described below.

FIG. 6 is a partially cutaway side view showing a cathode ray tube manufactured on the basis of the present invention. A cathode ray tube 60 has an airtight glass envelope 61 which has an evacuated interior. The envelope 61 has a neck 62 and a cone 63 continuously extending from the neck 62. In addition, the envelope 61 has a faceplate 10 sealed by a first glass. An explosion-proof tension band 65 consisting of a metal is wound around the periphery of the side wall of the faceplate 10. An electron gun 66 for emitting electron beams is arranged in the neck 62. A phosphor screen 67 is formed on the inner surface of the faceplate 10. The phosphor screen 67 is constituted by an optical filter layer and a phosphor layer formed thereon, which is excited by electron beams from the electron gun 66 to emit light. A deflection unit (not shown) is arranged outside the cone 63. The deflection unit serves to deflect electron beams to scan over the phosphor screen.

FIG. 7 is a view for explaining the structure of the phosphor screen 67.

A phosphor screen which is obtained by forming phosphor layers on, e.g., the filter substrate of Example 1, 2, or

3. can be used as the phosphor screen 67. As shown in FIG. 7, red, green, and blue emission phosphor layers RP, GP, and BP having emission colors corresponding to the red, green, and blue filters RF, GF, and BF consisting of the fine particle pigment layers are formed in the corresponding holes between the black matrices BM. The transmittance of the faceplate 10 serving as a transparent substrate is about 90%. A clear faceplate is used.

According to the color cathode ray tube having the above phosphor screen, the emission brightness levels of the phosphor layers RP, GP, and BP are proportional to the transmittances of the color filters RF, GF, and BF, respectively. In addition, since the faceplate is also clear, attenuation of the emission components of the phosphors is minimized. On the other hand, the transmittance of each color filter is low for light except for the emission component of the corresponding phosphor. Light components of external light (incident in a upward direction on the substrate in FIG. 7) except for the emission component of each phosphor, e.g., light components except for red color light, are attenuated in the red filter RF in proportion to the square of the low transmittance. Therefore, the reflected components of the external light are attenuated by the corresponding color filters, thereby increasing the contrast.

Since the red, green, and blue fine particle pigment layers having an average particle size of 0.01 to 0.2  $\mu\text{m}$  are formed on the substrate side of the black pigment particles having an average particle size of 0.2 to 5  $\mu\text{m}$ , irregular reflection is reduced at the boundary with the substrate. Even if the transmittance of the substrate is increased, components irregularly reflected by the black pigment particles can be reduced, thereby preventing a decrease in contrast.

The effect of the filters on the front surfaces of the phosphor layers can be maximized.

In the phosphor screen of this color cathode ray tube, phosphor layers may be formed in holes by the conventional method after a black matrix is formed in each example described above.

Additional advantages and modifications will readily occur to those skilled in the art. Therefore, the invention in its broader aspects is not limited to the specific details, representative devices, and illustrated examples shown and described herein. Accordingly, various modifications may be made without departing from the spirit or scope of the general inventive concept as defined by the appended claims and their equivalents.

What is claimed is:

1. A display screen comprising:

a transparent substrate having an inner surface and an outer surface; optical filter layers each containing color pigment particles having an average particle size of 0.2  $\mu\text{m}$  or less and each formed on said inner surface of said transparent substrate as rectangular or circular dots or stripes, the optical filter layers each having a first surface which faces the said inner surface of said transparent substrate and each having a second surface respectively opposite to each said first surface;

a black matrix layer containing black pigment particles having an average particle size of 0.2 to 5  $\mu\text{m}$  and at least a part of which is formed on each said second surface of said optical filter layers formed to cover

peripheral regions of said filter layers except for central portions thereof; and

5 phosphor layers formed on said optical filter layers and having an emission color corresponding to a color of a pigment contained in said optical filter layers.

2. A screen according to claim 1, wherein said optical filter layers include a red optical filter layer containing red pigment particles, a blue optical filter layer containing blue pigment particles, and a green optical filter layer containing green pigment particles.

10 3. A screen according to claim 1, wherein gaps between said filter layers are buried with black pigment particles.

15 4. A screen according to claim 1, wherein said optical filter layers are formed without any gap.

5. A method of manufacturing a display screen, comprising the steps of:

providing a transparent substrate having an inner surface and an outer surface;

20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055 100

coating a resist solution on a substrate to form a resist film  
prior to coating of a first color pigment dispersion;  
exposing and developing said resist film to form a resist  
film pattern in a region where said second color optical  
filter layer is to be formed;  
coating the first pigment dispersion on said resist film  
pattern and drying the first pigment dispersion to form  
a coating film;  
coating a resist decomposition agent on said first pigment  
dispersion coating film to remove said resist film pat-

tern and said first color pigment dispersion coating film  
formed thereon in the region where said second color  
optical filter layer is to be formed, thereby exposing  
said substrate in the region;  
coating a second pigment dispersion on the exposed  
substrate to form a coating film; and  
exposing and developing the coating film to pattern said  
second color optical filter layer.

\* \* \* \* \*